

Sept. 27, 1949.

P. G. CHACE

2,482,900

CORROSION-RESISTING COMPOSITE METAL

Original Filed June 23, 1941



Paul G. Chace  
Inventor  
Haynes and Koenig  
Attorneys

## UNITED STATES PATENT OFFICE

2,482,900

CORROSION-RESISTING COMPOSITE  
METAL

Paul G. Chace, Attleboro Falls, Mass., assignor to  
Metals and Controls Corporation, Attleboro,  
Mass., a corporation of Massachusetts

Original application June 23, 1941, Serial No.  
399,398, now Patent No. 2,366,178, dated Janu-  
ary 2, 1945. Divided and this application No-  
vember 11, 1944, Serial No. 563,016

13 Claims. (Cl. 29—195.5)

1

This invention relates to composite metal ele-  
ments and particularly to bimetallic elements  
which are corrosion-resisting.

This application is a division of my co-pending  
application, Serial No. 399,398, filed June 23, 1941,  
Patent 2,366,178.

Among the several objects of the present in-  
vention are the provision of a composite thermo-  
static metal which is corrosion-resisting, which  
has an improved bond, and which has a long life  
when operating in corrosion-promoting atmos-  
pheres and mediums; the provision of composite  
thermostatic metal of the class described which  
has both good hot-rolling and good cold-rolling  
properties; and the provision of composite ther-  
mostatic metal of the type indicated which is  
relatively simple and economical to manufacture.  
Other objects will be in part obvious and in part  
pointed out hereinafter.

The invention accordingly comprises the in-  
gredients and combinations of ingredients, the  
proportions thereof, and features of composition,  
which will be exemplified in the products herein-  
after described, and the scope of the application  
of which will be indicated in the following claims.

In the accompanying drawing in which is illus-  
trated one of various possible embodiments of the  
invention, the single figure is a representation of  
a bimetallic element showing a strip of iron chro-  
mium alloy fused throughout its length to a sim-  
ilar strip of copper silicon alloy.

Many of the thermostatic elements commonly  
in use are subject to corrosion when used in the  
presence of moisture in places such as steam radi-  
ators, or water mixing valves, or in other installa-  
tions where corrosion-promoting fluids or atmos-  
pheres come in contact with the thermostatic  
metal. As a result, such elements frequently need  
replacing, and inasmuch as corrosion tends to re-  
duce their activity in life, such corrosion may set  
up, unknown to the user, dangerous conditions  
which might result in loss of life or injury. To  
avoid this corrosion of the composite metal ele-  
ment, it has sometimes been customary in the  
past to treat the thermostatic metal surface to  
make it less subject to corrosion, as by plating it  
with a corrosion-resisting material, such as cad-  
mium, tin, zinc, lead, or chromium. This, how-  
ever, has the disadvantage that the plating in-  
creases the cost materially and does not assure  
satisfactory life for the thermostatic element.  
Furthermore, such plating is not entirely satis-  
factory since an electro-voltaic potential may be  
set up which produces pitting and eating away of  
the protective metal.

2

It has sometimes been the practice in the past  
to make a composite metallic element from an  
iron alloy having a high chromium content, and a  
metal alloy having a higher coefficient of expan-  
sion. The metal used for the high coefficient of  
expansion side has been one of the brasses. The  
mechanical properties of these brasses have pre-  
sented manufacturing difficulties, which in many  
instances have prevented the manufacture of an  
adequate and satisfactory composite metal. For  
example, the cold-working properties of brass are  
so different from those of the chromium iron  
alloy that it has been difficult to satisfactorily  
cold-work the metal after it has been put to-  
gether to form a thermostatic bimetal. More-  
over, it is highly advantageous in the manufac-  
ture of bimetal to hot-roll the material down  
from its thick ingot size to an intermediate stage.  
The brasses are not adapted to this, since their  
hot-rolling temperatures differ too much from  
that of the chromium iron alloy. The manufac-  
ture of the brass-chrome iron bimetal has there-  
fore been a relatively expensive process compared  
to the manufacture of bimetal in accordance with  
the present invention. The ingot size of the  
brass-chrome iron bimetal must be kept small  
because of the aforementioned difficulties and  
properties.

Where other constituents have been proposed  
for corrosion-resisting bimetals, it has been found  
relatively impossible to directly bond the metals  
together. For this reason, an intermediate solder  
layer has been used which led to two serious dis-  
advantages. First, the use of the solder layer  
decreases the corrosion-resisting property of the  
thermostatic metal due to inferior bonding, and  
second, the solder layer decreases the strength  
of the metal at elevated temperatures, since the  
solder bond is relatively weak. Also, solder-bonded  
material is difficult to hot-roll satisfactorily.

By the present invention, it is possible to ac-  
complish a direct bond between the metals, and  
they may be hot-rolled or cold-rolled in the de-  
sired manner. Their manufacture is accordingly  
economical, and a highly corrosion-resisting ther-  
mostatic metal is obtained.

According to the present invention a thermo-  
static element is provided which is corrosion-re-  
sisting per se, particularly to air, water and water  
vapor, thus eliminating the need for surface plat-  
ing. In addition, the present invention provides  
a thermostatic element made of composite ther-  
mostatic metal of the corrosion-resisting type  
which has a direct bond between the layers  
55 thereof.

The thermostatic metal of the present invention comprises layers of metal firmly secured together over their entire areas by a direct bond. One of the layers, in the present invention, comprises a corrosion-resisting metal having a low coefficient of expansion. The other layer comprises a second corrosion-resisting metal having a relatively high coefficient of expansion.

For the metal having a low coefficient of expansion a high chromium content stainless iron is employed. The composition of this alloy may be as follows:

|           | Per cent  |
|-----------|-----------|
| Manganese | 0.2-0.6   |
| Carbon    | 0.01-0.2  |
| Chromium  | 12-20     |
| Silicon   | 0-1.5     |
| Copper    | 0-1.5     |
| Iron      | Remainder |

For the high expansion material an alloy of copper and silicon is employed. The composition of this alloy may be as follows:

|           | Per cent |
|-----------|----------|
| Copper    | 96-99    |
| Silicon   | 0.5-4    |
| Manganese | 0-1      |
| Tin       | 0-2.5    |

The composite thermostatic metal of which bimetal will be described as an illustrative embodiment may be formed in any of the customary manners. It is preferably formed in one of the ways described in my co-pending application, Serial No. 399,398, filed June 23, 1941, Patent 2,366,178, reference to which is hereby made.

Referring now to the drawing, the single figure illustrates a bimetallic element composed of the two alloys discussed above. Numeral 1 represents the copper silicon alloy while 3 is the iron chromium alloy.

The tensile strength and other mechanical properties of the copper silicon alloys described are sufficiently near to the same properties of the chrome-iron alloys that the two metals work well together and may be easily cold-worked. This makes the manufacture thereof more economical. As a result of obtaining a direct bond between the metals comprising the present invention, a thermostatic metal having a higher strength, greater activity, wider usable temperature range, longer life and better corrosion-resisting properties than the corrosion-resisting bimetals hitherto known, is obtained. Former metals allegedly designed to have these desirable properties have instead been relatively weak, corrode relatively easily, are more difficult to manufacture, and in general are not satisfactory.

As specific examples of alloys which may be advantageously employed in the present invention, the following examples are given. They are illustrative only:

#### Chrome-iron alloy

|           | Per cent |
|-----------|----------|
| Manganese | 0.4      |
| Carbon    | 0.05     |
| Chromium  | 16-20    |
| Iron      | Balance  |

#### Copper-silicon Alloy No. 1

|           | Per cent  |
|-----------|-----------|
| Copper    | 97-99     |
| Silicon   | 0.75-1.75 |
| Manganese | 0.2-1.0   |

#### Copper-silicon alloy No. 2

|           | Per cent |
|-----------|----------|
| Copper    | 97-98.5  |
| Silicon   | 1-2.5    |
| Manganese | .15-.35  |

#### Copper-silicon Alloy No. 3

|           | Per cent |
|-----------|----------|
| Copper    | 98       |
| Silicon   | 1.25     |
| Manganese | 0.75     |

Attention is directed to my copending applications, Serial Nos. 563,013, 563,014 and 563,015, all filed November 11, 1944.

In view of the above, it will be seen that the several objects of the invention are achieved and other advantageous results attained.

As many changes could be made in the above alloys without departing from the scope of the invention, it is intended that all matter contained in the above description shall be interpreted as illustrative and not in a limiting sense.

I claim:

1. A corrosion-resisting thermostatic metal composed of an iron alloy containing: manganese approximately 0.2-0.6%, carbon approximately 0.01-0.2%, chromium approximately 12-20%, and the balance iron; and a copper alloy containing: silicon approximately 0.5-4%, manganese approximately 0.15-1%, and the balance copper; the surfaces of said alloys being fused together at the junction.

2. A corrosion-resisting thermostatic metal composed of an alloy having essentially the following composition:

|           | Per cent  |
|-----------|-----------|
| Manganese | 0.4       |
| Carbon    | 0.05      |
| Chromium  | 12-16     |
| Iron      | Remainder |

and an alloy having essentially the following composition:

|           | Per cent  |
|-----------|-----------|
| Copper    | 97-99     |
| Silicon   | 0.75-1.75 |
| Manganese | 0.2-1.0   |
| Iron      | Remainder |

the surfaces of said alloys being fused together at the junction.

3. A corrosion-resisting thermostatic metal composed of an alloy having essentially the following composition:

|           | Per cent  |
|-----------|-----------|
| Manganese | 0.2-0.6   |
| Carbon    | 0.01-0.2  |
| Chromium  | 12-20     |
| Iron      | Remainder |

and an alloy having essentially the following composition:

|           | Per cent  |
|-----------|-----------|
| Copper    | 97-99     |
| Silicon   | 0.75-1.75 |
| Manganese | 0.2-1.0   |
| Iron      | Remainder |

the surfaces of said alloys being fused together at the junction.

4. A corrosion-resisting thermostatic metal composed of an alloy having essentially the following composition:

|           | Per cent  |
|-----------|-----------|
| Manganese | 0.4       |
| Carbon    | 0.05      |
| Chromium  | 16        |
| Iron      | Remainder |

## 5

and an alloy having essentially the following composition:

|           | Per cent  |
|-----------|-----------|
| Copper    | 97-99     |
| Silicon   | 0.75-1.75 |
| Manganese | 0.2-1.0   |

the surfaces of said alloys being fused together at the junction.

5. A corrosion-resisting thermostatic metal composed of an alloy having essentially the following composition:

|           | Per cent  |
|-----------|-----------|
| Manganese | 0.4       |
| Carbon    | 0.05      |
| Chromium  | 12-16     |
| Iron      | Remainder |

and an alloy having essentially the following composition:

|           | Per cent |
|-----------|----------|
| Copper    | 98       |
| Silicon   | 1.25     |
| Manganese | 0.75     |

the surfaces of said alloys being fused together at the junction.

6. A corrosion-resisting thermostatic metal composed of an alloy having essentially the following composition:

|           | Per cent  |
|-----------|-----------|
| Manganese | 0.4       |
| Carbon    | 0.05      |
| Chromium  | 16        |
| Iron      | Remainder |

and an alloy having essentially the following composition:

|           | Per cent |
|-----------|----------|
| Copper    | 98       |
| Silicon   | 1.25     |
| Manganese | 0.75     |

the surfaces of said alloys being fused together at the junction.

7. A corrosion-resisting thermostatic metal composed of an alloy having essentially the following composition:

|           | Per cent  |
|-----------|-----------|
| Manganese | 0.4       |
| Carbon    | 0.05      |
| Chromium  | 12-16     |
| Iron      | Remainder |

and an alloy having essentially the following composition:

|           | Per cent  |
|-----------|-----------|
| Copper    | 97-98     |
| Silicon   | 1-2.5     |
| Manganese | 0.15-0.35 |

the surfaces of said alloys being fused together at the junction.

8. A corrosion-resisting thermostatic metal composed of an alloy having essentially the following composition:

|           | Per cent  |
|-----------|-----------|
| Manganese | 0.2-0.6   |
| Carbon    | 0.01-0.2  |
| Chromium  | 12-20     |
| Iron      | Remainder |

and an alloy having essentially the following composition:

|           | Per cent  |
|-----------|-----------|
| Copper    | 97-98.5   |
| Silicon   | 1-2.5     |
| Manganese | 0.15-0.35 |

the surfaces of said alloys being fused together at the junction.

## 6

9. A corrosion-resisting thermostatic metal composed of an alloy having essentially the following composition:

|           | Per cent  |
|-----------|-----------|
| Manganese | 0.2-0.6   |
| Carbon    | 0.01-0.2  |
| Chromium  | 12-20     |
| Iron      | Remainder |

and an alloy having essentially the following composition:

|           | Per cent |
|-----------|----------|
| Copper    | 98       |
| Silicon   | 1.25     |
| Manganese | 0.75     |

the surfaces of said alloys being fused together at the junction.

10. A corrosion-resisting thermostatic metal composed of an alloy having essentially the following composition:

|           | Per cent  |
|-----------|-----------|
| Manganese | 0.4       |
| Carbon    | 0.05      |
| Chromium  | 16        |
| Iron      | Remainder |

and an alloy having essentially the following composition:

|           | Per cent  |
|-----------|-----------|
| Copper    | 97-98.5   |
| Silicon   | 1-2.5     |
| Manganese | 0.15-0.35 |

the surfaces of said alloys being fused together at the junction.

11. A corrosion-resisting thermostatic metal composed of an alloy having essentially the following composition:

|           | Per cent  |
|-----------|-----------|
| Manganese | 0.4       |
| Carbon    | 0.05      |
| Chromium  | 16-20     |
| Iron      | Remainder |

and an alloy having essentially the following composition:

|           | Per cent  |
|-----------|-----------|
| Copper    | 97-99     |
| Silicon   | 0.75-1.75 |
| Manganese | 0.2-1.0   |

the surfaces of said alloys being fused together at the junction.

12. A corrosion-resisting thermostatic metal composed of an alloy having essentially the following composition:

|           | Per cent  |
|-----------|-----------|
| Manganese | 0.4       |
| Carbon    | 0.05      |
| Chromium  | 16-20     |
| Iron      | Remainder |

and an alloy having essentially the following composition:

|           | Per cent  |
|-----------|-----------|
| Copper    | 97-98.5   |
| Silicon   | 1-2.5     |
| Manganese | 0.15-0.35 |

the surfaces of said alloys being fused together at the junction.

13. A corrosion-resisting thermostatic metal composed of an alloy having essentially the following composition:

|           | Per cent  |
|-----------|-----------|
| Manganese | 0.4       |
| Carbon    | 0.05      |
| Chromium  | 16-20     |
| Iron      | Remainder |

7  
and an alloy having essentially the following composition:

|           | Per cent |   |
|-----------|----------|---|
| Copper    | 98       |   |
| Silicon   | 1.25     | 5 |
| Manganese | 0.75     |   |

the surfaces of said alloys being fused together at the junction.

PAUL G. CHACE. 10

8  
UNITED STATES PATENTS

| Number    | Name     | Date          |
|-----------|----------|---------------|
| 1,650,951 | Matthews | Nov. 29, 1927 |
| 1,929,655 | Scott    | Oct. 10, 1933 |
| 1,936,397 | Jennison | Nov. 21, 1933 |
| 1,991,438 | Wohrman  | Feb. 19, 1935 |
| 2,075,014 | Bassett  | Mar. 30, 1937 |
| 2,157,149 | Smith    | May 9, 1939   |
| 2,327,500 | Chace    | Aug. 24, 1943 |

OTHER REFERENCES

Pp. 1000-1002 of The Making, Shaping & Treating of Steel, 5th ed., 1940, pub. by Carnegie-Illinois Steel Corp., Pittsburgh, Pa.

REFERENCES CITED

The following references are of record in the file of this patent: